

R. E. WINNE,  
METHOD OF PERFORATING GLASS,  
APPLICATION FILED OCT. 9, 1917.

1,289,993.

Patented Dec. 31, 1918.

Fig. 1.



Fig. 2.



Fig. 4.



Fig. 3.



Fig. 5.



Fig. 6.



Fig. 7.



Fig. 8.



Inventor:  
Roy E. Winne,  
by *Albert S. Davis*,  
His Attorney.

# UNITED STATES PATENT OFFICE.

ROY E. WINNE, OF SCHENECTADY, NEW YORK, ASSIGNOR TO GENERAL ELECTRIC COMPANY, A CORPORATION OF NEW YORK.

## METHOD OF PERFORATING GLASS.

1,289,993.

Specification of Letters Patent. Patented Dec. 31, 1918.

Application filed October 9, 1917. Serial No. 195,613.

To all whom it may concern:

Be it known that I, ROY E. WINNE, a citizen of the United States, residing at Schenectady, county of Schenectady, in the State 5 of New York, have invented certain new and useful Improvements in Methods of Perforating Glass, of which the following is a specification.

My present invention relates to a method 10 of perforating glass and especially to a method of making very small holes through glass to adapt it for use as a die.

The object of my invention is to provide a simple, efficient and inexpensive method 15 of making holes through glass whereby a plurality of holes of any desired size may be made simultaneously.

In carrying my invention into effect I 20 heat the glass which is to be perforated until it is plastic and then force through it a plurality of wires which are held in parallel and suitably spaced in relation to one another. The glass is then allowed to cool slightly and the wires are withdrawn before it has 25 become hard. If the wires are of a material which is not wet by the glass used they will leave in the glass smooth holes of the desired form.

The novel features which I believe to be 30 characteristic of my invention are set forth with particularity in the appended claims. The manner in which my invention may be carried into effect however, together with other objects and advantages thereof will 35 best be understood by reference to the following description taken in connection with the accompanying drawing in which Figure 1 is a perspective of a holder in which the wires to be used may be loosely assembled 40 in the proper relation; Figs. 2 and 3 are perspectives showing the manner in which the wires are fastened into a convenient holder so as to retain the proper relation to one another while the method is being carried out; Fig. 4 is a view of the completed 45 holder; Fig. 5 is a perspective, and Fig. 6 is a cross-section showing the relation of the holder to a die blank while the perforating operation is being carried out; Fig. 7 50 is a perspective of a completed die, and Fig. 8 is an enlarged cross-section through a portion of the die.

In proceeding to carry my invention into effect I first find it desirable to construct a 55 suitable holder for holding the wire and, in

case a plurality of holes are to be made simultaneously, retaining all of the wires in proper spaced relation to one another while they are forced through the glass. In constructing such a holder I first assemble the 60 wires 1 in holes 2 in the disk 3 which may be made of metal or refractory material. The holes are parallel with one another and spaced in the manner which is desired in the finished product. The disk 3 is then placed 65 in the conical opening 4 in the plate 5, both disk and plate resting upon the plate 6 of refractory material. The glass bead 7 on the stem 8 is then heated until it becomes plastic and forced down over the disk 3 70 until the ends of wires 1 are embedded in the glass. The whole assemblage may also be heated by the jet 9 to assist the operation of embedding the ends of the wires in the glass bead 7. The hooks 10 on the ends of the 75 wires assist in anchoring them firmly in the glass when it is cooled. The bead 7, in being forced down into the hole 4 is also molded into the conical shape indicated in Fig. 4. 80

In utilizing the holder thus constructed for making a die a glass blank is placed upon a plate 12 of graphite or other refractory material and heated to a temperature at which the bottom of the blank becomes 85 plastic. In the case of lead glass this temperature may be about 800° C. The holder is then inserted in the blank and the wires 1 are forced through the bottom. The blank is then allowed to cool slightly and the 90 holder and wires are withdrawn before the glass becomes hard, each wire leaving a clean hole through the glass. In the case of lead glass the temperature of the glass when the wires are withdrawn may be about 95 500° C.

In the case of ordinary glass, such for example as lead glass, I find that tungsten or molybdenum wire is especially suitable for making the perforations. This is probably due to the fact that the surface of the wire is not wet by the glass and that the wire does not give off gas when heated. Wires of tungsten or molybdenum also do not become as flexible at the temperature 100 at which the operation is carried out as wires of other metals. In case any gas was given off by the wire bubbles would be formed in the glass and the holes would be imperfect. 110

In some cases it is desirable that the hole through the glass shall be conical in form instead of cylindrical. The holes may be given a conical form as indicated in Fig. 8, 5 by proper manipulation of the apparatus employed. If the glass is heated to the right temperature the wire, when it is pressed down upon the glass, instead of immediately penetrating the surface will force the surface of the glass down and form a conical depression in the surface. As a result when 10 the wire finally penetrates the under surface of the glass the glass will touch it only at the point. If the heating is at once discontinued at this point the hole which is left 15 when the wire is withdrawn will have the shape indicated in Fig. 8. If it is desired that the hole be less conical or cylindrical in form the heating of the glass may be continued and the depression in the glass will gradually fill up until the wire is surrounded closely by the glass throughout the thickness of the glass.

While I have described my invention with 25 especial reference to perforating glass for making dies, it will be apparent that it is by no means limited to this particular application but will be of utility wherever it is desired to perforate glass for other purposes.

What I claim as new and desire to secure by Letters Patent of the United States is:

1. The method of making a hole through glass which consists in heating the glass un-

til it is plastic, forcing a tungsten wire 35 through the glass, while it is in that condition allowing the glass to partially cool and withdrawing the wire before the glass becomes hard.

2. The method of making a hole through 40 glass which consists in heating the glass until it is plastic, forcing through the glass while it is in that condition a wire composed of a metal which is not wet by the glass and which does not give off gas when heated, 45 allowing the glass to partially cool and withdrawing the wire before the glass becomes hard.

3. The method of making a hole through 50 lead glass which consists in heating it to a temperature of about 800° C., forcing a tungsten wire through the glass while it is in that condition, allowing the glass to cool to about 500° C. and then withdrawing the wire.

4. The method of making a glass die which consists in heating a glass blank until it is plastic, forcing through the glass while in that condition a plurality of tungsten wires which are held in parallel and 60 suitably spaced relation to one another, allowing the glass to partially cool and withdrawing the wires before the glass becomes hard.

In witness whereof, I have hereunto set 65 my hand this 8th day of October, 1917.

ROY E. WINNE.